

## UNITED STATES PATENT OFFICE

2,380,319

## PROCESS FOR TREATMENT OF CASHEW NUTSHELL LIQUID AND THE RESULTING PRODUCT

Roland E. Kremers, Summit, N. J., assignor to General Foods Corporation, Hoboken, N. J., a corporation of Delaware

No Drawing. Application May 4, 1942,  
Serial No. 441,758

12 Claims. (Cl. 260—521)

The present invention relates to the treatment of cashew nut shell liquid, and more particularly to an improved method of treating the liquid to convert it into a plastic product.

The principal object of the invention is to provide a method of converting cashew nut shell liquid of relatively high anacardic acid content into a plastic form which is adapted to be packed in inexpensive paper sacks or other suitable containers and which may be stored and/or shipped without undergoing any substantial change and which may be safely handled during shipment thereof.

Another object of the invention is to prevent contamination of cashew nut shell liquid of high anacardic acid content as a result of the corrosion which would otherwise occur if the liquid is shipped in metallic containers, by converting the liquid into a plastic form which is adapted to be shipped in paper or other suitable non-metallic containers or in metallic containers without being subject to the aforesaid contamination by corrosion.

A further object of the invention is to prevent the injury of handlers of cashew nut shell liquid during shipment thereof by converting the toxic vesicant liquid into a non-toxic, plastic state in which it may be safely handled.

A still further object of the invention is to convert cashew nut shell liquid into a plastic product by reacting said liquid with a sufficient amount of a suitable alkaline compound and from which the cashew nut shell liquid may be later recovered in approximately its original condition by suitable treatment of the solid product.

Another object of the invention is to provide a method of recovering cashew nut shell liquid from a plastic reaction product of cashew nut shell liquid and a suitable alkaline compound.

The necessity for improving the commercial methods for the storage and shipment of cashew nut shell liquid arises from the fact that the high quality liquid produced by modern extraction methods, and having an anacardic acid content of from 40% to 65% or 70%, unfortunately is liable to undergo spontaneous decomposition with the evolution of  $\text{CO}_2$ , thus building up an excessive pressure in the drums in which the liquid is shipped. This tends to cause loss of the liquid due to opening of the seams and sometimes bursting of the drums in which the liquid is stored and transported, and also may poison persons who come in contact with the toxic, vesicating oil through handling the leaky drums. Furthermore, the available supply of metals at times becomes limited.

Now, in accordance with the present invention, it has been found that the above-mentioned difficulties may be obviated and that cashew nut shell liquid of high anacardic acid content, say of at least 40%, may be converted into a plastic product, in which the anacardic acid is stabilized against decomposition by reacting it with a sufficient amount of an oxide or hydroxide of a suitable metal, and that the plastic product thus produced may be safely stored and shipped in non-metallic containers, such as paper bags, and that the cashew nut shell liquid may be recovered in approximately its original condition by reacting the plastic product with a suitable amount of a dilute acid. The cashew nut shell liquid may be treated directly with the oxide or hydroxide, or it may be converted by the addition of a small amount of water into a water-in-oil emulsion which may then be reacted with the oxide or hydroxide.

For purposes of illustration, but not by way of limitation, this invention is hereinafter described as practiced by reacting hydrated lime with cashew nut shell liquid. Generally, it has been found that the slaked lime used for the solidification of cashew nut shell liquid should not contain a high percentage of magnesium oxide or hydroxide if a desirable product is to be obtained. For example, in most instances, the amount of magnesia associated with the lime will not exceed about 15%. In general, the lower the magnesia content in the lime, the better will be the physical properties of the product. It will, of course, be understood that in place of hydrated lime, unslaked lime or oxides and hydroxides of the other alkaline earth metals, such as the oxides and hydroxides of barium and strontium, may be utilized.

In practicing the present invention, a sufficient quantity of lime is added either to the cashew nut shell liquid of high anacardic acid content or to an emulsion thereof to form a plastic mass which subsequently hardens. The amount of lime employed is in excess of that theoretically required to react with the anacardic acid of the cashew nut shell liquid to form the neutral salt, and the excess present may be varied to obtain a plastic product of the desired characteristics. For example, in the case of a liquid containing from 50% to 70% anacardic acid, the most desirable properties of the reaction product are obtained with an amount of lime included within the range of from about 12% to about 25% by weight of the liquid. If less than 12% of lime is used, the mixture will remain too fluid in tropical regions for

safe handling, while if more than 25% of lime is utilized, the cost of materials and the tendency of the mixture to solidify too rapidly will become serious factors.

It has been found that the addition of a small amount of water to the cashew nut shell liquid to form a water-in-oil emulsion prevents a premature setting of the mixture when lime is added to the liquid and provides a product which pours easily and is readily handled. In the absence of the added water, the lime-cashew nut shell liquid mixture may solidify before the lime can be thoroughly dispersed therein and the hardness of the product makes the emptying of the apparatus in which it is mixed more difficult. When an emulsion is reacted with the oxide or hydroxide, it is advantageously heated to a temperature above 50° C. 15

The reaction between lime and cashew nut shell liquid of high anacardic acid content is exothermic, so that the mixture becomes hot and remains fluid for a time and then sets on cooling. While the mixture is in the fluid stage, it may be poured into suitable containers, or after it has set, it may be transferred to suitable containers and made to conform to their shape by pressure. 20 25

While the reaction is preferably conducted in such a manner that the exothermic heat is utilized to accelerate the reaction, and the reaction mixture then cooled to room temperature to form the plastic mass, it is to be understood that the reaction may be conducted at substantially room temperature, if so desired, by cooling during the progress of the reaction, or by adding the ingredients slowly. 30 35

After storage and/or shipment of the solid product, produced by the above-described reaction, the cashew nut shell liquid may be recovered therefrom in approximately its original condition by removing the metal combined with the anacardic acid by reaction thereof with a dilute mineral acid, say a 5% or 10% sulphuric, hydrochloric, or phosphoric acid, or a dilute organic acid, such as oxalic or tartaric. It is preferred to use an acid which will form a water-insoluble salt with the metal in the product. At room temperature, the reaction proceeds rapidly at the surface of the solid, but the released liquid promptly forms a coating over the unreacted residue, which stops the progress of the reaction. This stoppage can be prevented by raising the temperature of the mixture to about 50° C. to about 70° C. and agitating vigorously to break the oil film, or by adding to the mixture a solvent for cashew nut shell liquid, preferably one which is immiscible with water, such as hexane, benzene, carbon tetrachloride, trimethyllethane, or chloroform. The original or recovered cashew nut shell liquid may also be used as a solvent for this purpose. The first procedure, namely, the one employing vigorous agitation without solvent, exposes the unreacted particles by emulsifying the liberated cashew nut shell liquid, whereas, the second procedure, namely, the one which employs a solvent, exposes the unreacted particles by dissolving away the liberated cashew nut shell liquid. Temperatures employed and dilutions of the acids will vary with the composition of the product being treated. In general, temperatures employed should be below 100° C. and the acids used as dilute as permitted by the necessity of obtaining complete removal of the lime and of minimizing the size of equipment required. The purpose of these precautions is to

avoid the well known polymerization and decarboxylation of cashew nut shell liquid. The product so treated, that is the entire reaction mixture, contains cashew nut shell liquid, dilute acid, with a calcium salt, which is soluble or insoluble, depending on the acid employed. These constituents may be separated in any suitable manner, as by centrifuging, filtering, or decantation.

The following specific examples will serve to illustrate and explain the present invention, and more particularly the formation of the lime-cashew nut shell liquid reaction product and the subsequent recovery of cashew nut shell liquid therefrom.

### *Example 1*

60 grams of slaked lime ( $\text{Ca}(\text{OH})_2$ ) is placed in a suitable receptacle and is reacted with 300 grams of cashew nut shell liquid, having an anacardic acid content of approximately 65%, by adding  $\frac{1}{3}$  of the cashew liquid to it in several portions, each of which is stirred in vigorously until a smooth paste has been formed. Then the remainder of the cashew nut shell liquid is added and incorporated into the paste. Considerable heat is evolved in the preliminary step of the reaction. The final mass remains soft for a time and then gradually hardens as it cools to room temperature. This transition continues after the mass has cooled. During the soft stage, the mass can be transferred to suitable containers and made to conform to their shape by the application of pressure thereto. The final product has about the texture and hardness of a chilled chocolate liquor, and like the latter, can be readily chipped or grated, or otherwise comminuted.

### Example 2

22 grams of slaked lime ( $\text{Ca}(\text{OH})_2$ ) is reacted with 200 grams of cashew nut shell liquid having an anacardic acid content of approximately 65% in the manner described above in Example 1, except that the reaction was somewhat accelerated by warming the plastic mass to a temperature of about 65° C. to 70° C. While still warm, the mass flows under its own weight and when poured into a bag will automatically conform to its shape. In fact, the product retains a considerable degree of plasticity during its storage.

Ratios of the reactants intermediate between those of Examples 1 and 2 will give products with intermediate properties.

### *Example 3*

## Recovery of cashew nut shell liquid from the solidified product.

140 grams of solidified cashew nut shell liquid containing 20% of added  $\text{Ca}(\text{OH})_2$  were reduced to shavings, covered with 250 cubic centimeters of water and agitated with a motor driven stirrer. 40 grams of sulphuric acid diluted with 130 cubic centimeters of water were slowly added to the subdivided material. The temperature of the material was slowly raised to 65° C.-70° C. and after 2 hours, the resultant emulsion was broken by suction filtration. The supernatant oil was separated and washed repeatedly with warm water until excess acid had been removed. The recovered oil was then dried over anhydrous sodium sulphate.

The procedure for using a solvent, such as those previously mentioned, is similar, and the solution is separated from the insoluble material. Subsequently, the dried solution must be distilled to remove the solvent. When the reaction is carried out on a commercial scale, regenerated

cashew nut shell liquid may be used as a solvent and at the end of each cycle, an appropriate quantity removed from the system in accordance with well established engineering principles.

*Example 4*

In the following example, a preferred method of conducting the reaction between cashew nut shell liquid and slaked lime is described.

Sufficient water is added to cashew nut shell liquid having an anacardic acid content of approximately 60% to bring the moisture content of the liquid up to five percent. The liquid is then heated to a temperature of 60° C. with sufficient stirring to disperse the water thoroughly in the liquid and to form a water-in-oil emulsion. An amount of slaked lime equal to seventeen percent of the weight of the liquid is then added to the emulsion and the latter is stirred vigorously. The mixing is continued for five minutes, during which the temperature rises to about 90° C., and the plastic material is then poured into molds to cool.

The amount of slaked lime used in the above example is one hundred and forty percent in excess of the amount theoretically necessary to react to form the neutral salt with the anacardic acid of the liquid, assuming that the slaked lime is ninety-one percent calcium hydroxide and the cashew nut shell liquid is sixty percent anacardic acid. The amount of lime used should be varied in accordance with the calcium hydroxide content of the lime and the acid content of the oil.

It will be noted in the above example that after the water was added to the cashew nut shell liquid, the latter was heated to 60° C. It has been found that at temperatures below 50° C., the greater viscosity of the liquid inhibits the dispersion of lime therein and the reaction between the ingredients is slow and often incomplete.

*Example 5*

In the following example, a method of regenerating anacardic acid from the plastic product herein described by the use of oxalic acid and an organic solvent is described.

A mixture of 111 grams of calcium hydroxide and 650 grams of an emulsion of cashew nut shell liquid are prepared according to the method described in Example 4. When cool, this product is leached at room temperature with acetone until practically free from soluble material. The acetone-wet solid is treated with a solution of 205 grams of oxalic acid in one liter of acetone and the mixture is stirred for one hour while it is heated to a temperature just below its boiling point. The solution is then filtered and the residue is washed with two portions of 200 cubic centimeters each of acetone. The filtrate is then concentrated by distillation and the final traces of acetone are removed under vacuum. The resulting liquid, upon cooling, precipitates a small amount of crystalline oxalic acid which may be removed by filtration. The yield of anacardic acid is 317 grams, 91.7% pure, which is 74% of theory. The process results in the separation of the phenolic components of the cashew nut shell liquid from the anacardic acid, and this method of regenerating the anacardic acid from the plastic product is not claimed specifically herein since the process of separating the phenolic components from anacardic acid is the subject matter of copending application Serial No. 533,409 filed April 29, 1944.

While the above examples described the use of slaked lime, unslaked lime may also be employed, but the reaction of lime with cashew nut shell liquid of high anacardic acid content is more rapidly effected with slaked lime, the use of which is, therefore, preferred. The lime undoubtedly reacts with the anacardic acid of the liquid and may also react with other constituents of the liquid, although this is not definitely known. The lime must be used in sufficient amount to produce a plastic product in which the anacardic acid is stabilized against decomposition as a result of its conversion at least in part into one or more of its calcium salts. The product formed is a material from which cashew nut shell liquid can be readily liberated and which will not undergo decomposition during storage and shipment thereof. However, the plasticity of the reaction product decreases with an increasing amount of lime.

Generally, with cashew nut shell liquid having from 40% to 70% anacardic acid content, it is essential to use an excess of the theoretical quantity of lime based upon that required to react with the anacardic acid to form a neutral salt thereof. Also, as the anacardic acid content of the cashew nut shell liquid increases, the relative amount of lime required to obtain a given degree of plasticity decreases.

Anacardic acid has the following structural formula:



in which the  $\text{C}_{15}\text{H}_{27}$  is an open, unsaturated hydrocarbon chain containing two double bonds (i. e., four unsaturated carbon atoms). The decarboxylation of anacardic acid (i. e., the loss of  $\text{CO}_2$  from its contained carboxyl group) yields the following phenol known as anacardol:



This phenol is probably present in some proportion in the cashew shell, but owes its presence in oils of commerce largely to its formation from anacardic acid.

Commercial oils obtained by the old methods of heat extraction have most of the anacardic acid originally contained in the shell converted into anacardol by the high temperature treatment employed for extraction. According to the literature, the percentage of anacardic acid in heat-extracted oils is not substantially greater than 16%, for example, see the article by Harvey and Caplan in "Industrial and Engineering Chemistry," October, 1940, "Cashew nut shell liquid," pages 1306 to 1310. On the other hand, the oils which may now be obtained by the simple method of pressure extraction are known to contain as much as 70% anacardic acid.

It is to be understood that the invention is applicable to cashew nut shell liquid having anacardic acid present in proportions greater than 70%.

The method of the present invention for the stabilization of cashew nut shell liquid on storage and shipment does not apply to the heat-extracted oils. These may also be stabilized against gas evolution by reaction with lime, but the need for their stabilization is not nearly so great as in the case of the high anacardic acid-containing oils obtained by pressure extraction of cashew shells. Besides, the heat-extracted oils do not yield the solid reaction product of the present invention. Recent tests carried out on a series of oils containing varying percentages of anacardic acid show that the solid reaction product of the present invention requires the use of cashew nut shell liquid having an anacardic acid content of at least 40%. The reaction products obtained with cashew nut shell liquids containing less than this percentage of anacardic acid are free-flowing masses incapable of being packed in paper containers.

Anacardic acid is theoretically capable of producing the following calcium salts by reaction with one or two equivalents of alkali:

(1) Neutral salt— $(C_{22}H_{31}O_3)_2Ca$



(2) Basic salt— $C_{22}H_{30}O_3Ca$



(3) Basic salt— $C_{22}H_{32}O_4Ca$



All three of these anacardates may be present in the reaction product with lime.

It is not an object to prepare any of these salts as such, but to keep them in contact with the remainder of the cashew nut shell liquid constituents in order to confer desirable properties on the mixture. There appears to be a marked degree of mutual solubility between the products formed since in a properly formed mixture, unreacted specs of lime are the only evident signs of lack of homogeneity.

The plastic character of the reaction product of the present invention which adapts it for storage and shipment is an important advantage. For example, the plastic product is unlikely to poison persons coming in contact with it because of its inability to enter the pores of the skin. Moreover, it may be stored and shipped in ordinary paper bags or other inexpensive containers without decomposition or loss of constituents by bleeding. It may be shipped in metal containers, in which case all effects of corrosion formerly produced by storage and shipment in metallic containers are eliminated, thus preventing con-

tamination of the product with foreign matter.

While the invention has been described in detail with specific examples, such examples are illustrative and are not given as limitations, since other modifications within the spirit and scope of the invention will be apparent to those skilled in the art. Hence, the invention is to be understood as limited only as indicated in the appended claims, in which the intent is to set forth all the novelty over the prior art.

I claim as my invention:

1. The method of converting cashew nut shell liquid containing the usual non-acidic constituents of cashew nut shell liquid and having an anacardic acid content of from at least 40% to about 70% into a hardened plastic product capable of being stored and shipped without substantial loss thereof due to decomposition or loss of constituents by bleeding which comprises mixing and reacting said cashew nut shell liquid with an alkaline earth metal compound selected from the group consisting of an oxide and a hydroxide in an amount in excess of that theoretically required to form a neutral alkaline earth metal salt of the anacardic acid content of said liquid, forming and hardening the product of said reaction into a hardened plastic product of sufficient bulk to prevent appreciable air-oxidation of the product, said product being capable of regenerating cashew nut shell liquid in substantially unoxidized condition upon treatment of said product with an acid capable of forming a salt with the alkaline earth metal of the product.

2. The method of claim 1 wherein the alkaline earth metal compound is a calcium compound selected from the group consisting of slaked and unslaked lime.

3. The method of claim 1 wherein the cashew nut shell liquid treated has an anacardic acid content of from 50% to 70% and wherein the alkaline earth metal compound is a calcium compound selected from the group consisting of slaked and unslaked lime and is present from about 12% to about 25% by weight of the cashew nut shell liquid.

4. The method of converting cashew nut shell liquid containing the usual non-acidic constituents of cashew nut shell liquid and having an anacardic acid content of from at least 40% to about 70% into a hardened plastic product capable of being stored and shipped without substantial loss thereof due to decomposition or loss of constituents by bleeding which comprises forming a water-in-oil emulsion of said cashew nut shell liquid, mixing and reacting said emulsion with an alkaline earth metal compound selected from the group consisting of an oxide and a hydroxide in an amount in excess of that theoretically required to form a neutral alkaline earth metal salt of the anacardic acid content of said liquid, forming and hardening the product of said reaction into a hardened plastic product of sufficient bulk to prevent appreciable air-oxidation of the product, said product being capable of regenerating cashew nut shell liquid in substantially unoxidized condition upon treatment of said product with an acid capable of forming a salt with the alkaline earth metal of the product.

5. The method of claim 4 wherein the cashew nut shell liquid treated has an anacardic acid content of from 50% to 70%, wherein the alkaline earth metal compound is a calcium compound selected from the group consisting of slaked and unslaked lime and is present from

65

about 12% to about 25% by weight of the cashew nut shell liquid, and wherein the reaction is conducted at a temperature of at least 50° C.

6. A hardened plastic product of sufficient bulk to prevent appreciable air oxidation thereof and capable of being stored and shipped without substantial loss thereof due to decomposition or loss of constituents by bleeding comprising the reaction product of cashew nut shell liquid containing the usual non-acidic constituents of cashew nut shell liquid and having an anacardic acid content of from at least 40% to about 70% and an alkaline earth metal compound selected from the group consisting of an oxide and a hydroxide in an amount in excess of that theoretically required to form the neutral alkaline earth metal salt of the anacardic acid content of said liquid, said product being capable of regenerating cashew nut shell liquid in substantially unoxidized condition upon treatment of said product with an acid capable of forming a salt with the alkaline earth metal of the product.

7. The product of claim 6 wherein the alkaline earth metal compound is a calcium compound selected from the group consisting of slaked and unslaked lime.

8. The product of claim 6 wherein the cashew nut shell liquid treated has an anacardic acid content of from 50% to 70% and wherein the alkaline earth metal compound is a calcium compound selected from the group consisting of slaked and unslaked lime and is present from about 12% to about 25% by weight of the cashew nut shell liquid.

9. A hardened plastic product of sufficient bulk to prevent appreciable air oxidation thereof and capable of being stored and shipped without substantial loss thereof due to decomposition or loss of constituents by bleeding comprising the reaction product of a water-in-oil emulsion of cashew nut shell liquid containing the usual non-acidic constituents of cashew nut shell liquid and having an anacardic acid content of from at least 40% to about 70% and an alkaline earth metal compound selected from the group consisting of an oxide and a hydroxide in an amount in excess of that theoretically required to form the neutral alkaline earth metal salt of the anacardic acid

content of said liquid, said product being capable of regenerating cashew nut shell liquid in substantially unoxidized condition upon treatment of said product with an acid capable of forming a salt with the alkaline earth metal of the product.

10. The product of claim 9 wherein the cashew nut shell liquid treated has an anacardic acid content of from 50% to 70% and wherein the alkaline earth metal compound is a calcium compound selected from the group consisting of slaked and unslaked lime and is present from about 12% to about 25% by weight of the cashew nut shell liquid.

11. The method of converting cashew nut shell liquid containing the usual non-acidic constituents of cashew nut shell liquid and having an anacardic acid content of from at least 40% to about 70% into a hardened plastic product capable of being stored and shipped without substantial loss thereof due to decomposition or loss of constituents by bleeding which comprises mixing and reacting said cashew nut shell liquid with an alkaline earth metal compound selected from the group consisting of an oxide and a hydroxide in an amount in excess of that theoretically required to form a neutral alkaline earth metal salt of the anacardic acid content of said liquid, forming and hardening the product of said reaction into a hardened plastic product of sufficient bulk to prevent appreciable air-oxidation of the product, said product being capable of storage and shipment without substantial loss thereof and of regenerating cashew nut shell liquid in substantially unoxidized condition upon treatment of said product with an acid capable of forming a salt with the alkaline earth metal of the product.

12. The process of claim 11 wherein the alkaline earth metal compound is a calcium compound selected from the group consisting of slaked and unslaked lime.

ROLAND E. KREMERS.